

I. HECHENBLEIKNER.  
APPARATUS AND PROCESS FOR OXIDIZING PHOSPHORUS.

APPLICATION FILED NOV. 6, 1914.

1,167,755.

Patented Jan. 11, 1916.



Witnesses:

J. W. Wells  
A. De Mott

Inventor  
Ingenieur Hedenbleikner  
By his Attorneys

Meyers, Cushman & Rea

# UNITED STATES PATENT OFFICE.

INGENUIN HECHENBLEIKNER, OF CHARLOTTE, NORTH CAROLINA.

## APPARATUS AND PROCESS FOR OXIDIZING PHOSPHORUS.

1,167,755.

Specification of Letters Patent. Patented Jan. 11, 1916.

Application filed November 6, 1914. Serial No. 870,625.

*To all whom it may concern:*

Be it known that I, INGENUIN HECHENBLEIKNER, a subject of the Emperor of Austria-Hungary, residing at Charlotte, in the 5 county of Mecklenburg and State of North Carolina, have invented new and useful Improvements in Apparatus and Processes for Oxidizing Phosphorus, of which the following is a specification.

10 This invention relates to the manufacture of phosphorus pentoxid and it is particularly applicable in the production of phosphorus from phosphatic material such as phosphate rock. In the production of phosphorus from such a phosphatic material, the phosphatic material together with a suitable flux and a carbonaceous material is heated to a very high temperature in an electric furnace, the effect being to drive off oxidizable gases including phosphorus and the phosphorus gas is afterward oxidized to phosphorus pentoxid. These gases which pass from the furnace have a very high temperature and are also capable of developing 25 a further amount of heat by their oxidation.

My invention resides in the novel process and also in the novel apparatus to be described hereinafter.

One of the objects of my invention is to 30 provide a process and apparatus which will operate to utilize the heat contained in these gases or developed by their oxidation so as to pre-heat a charge or portion of the charge before it is fed into the furnace.

35 A further object of the invention is to provide a process and apparatus which will operate to insure a thorough heating of all parts of the charge before it passes into the furnace.

40 A further object of the invention is to provide a process and apparatus which will insure a thorough oxidation of the oxidizable gases as they pass through the charge.

Further objects of the invention will appear 45 hereinafter.

The invention consists in those features of my process and apparatus hereinafter described, all of which contribute to produce an efficient process or apparatus for producing phosphorus pentoxid.

A preferred embodiment of my invention will be particularly described in the following specification while the broad scope of my invention will be pointed out in appended claims.

In the drawings the figure is a side ele-

vation in partial section through the preferred embodiment of my apparatus, and which is preferably employed for practising my novel process.

Referring more particularly to the parts, 1 represents a furnace which is preferably an electric furnace of any suitable type. The furnace illustrated has a conical dome 2 through which electrodes 3 pass into the 65 interior and any suitable means is provided for causing an electric current to pass between the electrodes within the furnace. The upper end of the furnace is preferably provided with an up-take 4 which is preferably in the form of an elbow in order to facilitate the practising of my invention.

The furnace is supplied with a phosphate rock preferably in the form of calcium phosphate, a suitable flux such as silica, and a 75 carbonaceous material such as carbon, charcoal or coke. The reaction which takes place in the furnace is substantially as follows:



From an inspection of this formula, it is apparent that oxidizable gases pass out of the furnace in the form of carbon monoxide 85 and phosphorus. Furthermore, these gases are at a very high temperature.

According to my process and apparatus, I employ the sensible heat and the calorific power of these gases to raise the temperature of the incoming charge which is to be introduced into the furnace, and I preferably exclude from the charge which is heated by the gases, the carbonaceous material so as to prevent its combustion and to insure 95 its being delivered into the furnace.

According to my invention I prefer to provide means for holding a charge of material exclusive of the carbonaceous material and arranged so as to pass the gases through 100 the mass of this charge, and also arranged so that the charge progresses slowly toward the furnace in a continuous stream. I pass the gases in a current through this charge and agitate the charge so as to effect a thorough heating thereof.

The holder for the charge referred to is preferably in the form of a duct 9 which is preferably slightly inclined and which connects to the end of the elbow 5, said duct 110 being preferably lined with a refractory fire-brick and having a covering or shell 8

of suitable metal. The elbow 5 is preferably similarly constructed out of refractory fire-brick and metal.

I provide means for feeding the phosphatic material and the flux or silicious material into the upper end of the duct. This is most conveniently accomplished by providing a feed hopper 16 in a fixed neck 14 connecting with the upper end of the duct. The delivery opening from the hopper 16 is arranged so that the material falls by gravity into the upper end of the duct. While the charge is in the holder or duct 9, I prefer to agitate it so as to insure a thorough heating of the same by the gases which pass upwardly through the elbow 5 and through the duct. This is preferably accomplished by rotating the duct on its longitudinal axis. For this purpose the weight of the duct is preferably taken on a suitable frame 12, the upper part of said frame being provided with rollers 10 receiving rings 10<sup>a</sup> on the exterior of the duct. These rollers are preferably flanged and form a cradle to hold the tubular duct in position. The duct is also provided with an encircling gear wheel 11<sup>a</sup> with which meshes a pinion 11, said pinion being driven by any suitable gearing 11<sup>b</sup>. The interior of the duct is preferably provided with longitudinal ribs 13 formed in the fire-brick. The charge being in a finely divided state as this duct rotates, the material is being constantly carried up on the ascending side of the duct and falls back toward the bottom. In this way a very thorough mixture of the charge takes place and a thorough heating by the gases passing through the duct. Such an arrangement as this will operate to extract a large portion of the sensible heat of these gases, but I prefer also to utilize the calorific power of the gases so as to benefit by the heat developed and also burn the phosphorus to its pentoxide ( $P_2O_5$ ). For this purpose, I prefer to provide inlet openings 7 which are preferably in the upper side of the elbow, and through these air or oxygen passes inwardly; the inward draft at this point is caused by the velocity of the gases passing outwardly from the elbow. The carbonaceous material is preferably fed into the furnace through the upper side of the elbow through the medium of a suitable charging hopper 6. In other words, I provide means for separately or independently feeding the carbonaceous material to the furnace in such a way that it is not passed through the duct 9.

Although the charge in the duct is preferably in a finely divided state, it is preferably as free from dust as possible, but in order to remove all the dust possible after the gases pass from the duct, I prefer to provide a dust collector of any suitable type, such as indicated at 15. The dust col-

lector illustrated is of a simple upright cylindrical form, the middle of the dust chamber within the same being provided with a baffle wall 17 which directs the current of gases downwardly so that they pass under 70 the lower edge of the baffle plate and upwardly on the opposite side. The momentum of the dust in the downwardly directed current causes the dust to collect at the bottom of the chamber. The upper side of the dust collector can be provided with a suitable outlet pipe 19 which may connect with a suitable exhaust fan 20 which delivers the exhaust gases through a suitable pipe 21.

It is understood that I may employ any 80 suitable type of dust collectors, the one illustrated being simply by way of example.

As the gases pass through the duct, they mix with the oxygen or air which is admitted by the air inlets 7 so that the carbon monoxid and the phosphorus in the gases become oxidized according to the following formulae:



It is understood that the embodiment of the invention described herein is only one of the many embodiments or forms my invention may take, and I do not wish to be limited in the practice of my invention, nor in my claims to the particular embodiment set forth.

What I claim is:—

1. The process of manufacturing phosphoric acid which consists in heating together in a furnace phosphatic material, a flux and a carbonaceous material, feeding and conducting a mass of the phosphatic material, and the flux toward the furnace, passing the gases from said furnace through said mass as it progresses toward the furnace to pre-heat the same, and separately feeding the carbonaceous material into the furnace.

2. The process of manufacturing phosphoric acid which consists in heating together in a furnace phosphatic material, a silicious flux and a carbonaceous material, feeding and conducting a stream of the phosphatic material and the flux toward the furnace, passing the gases from the furnace through said stream as it progresses toward the furnace to pre-heat the same, and separately feeding the carbonaceous material into the furnace.

3. The process of manufacturing phosphoric acid which consists in heating together in a furnace phosphatic material, a flux and a carbonaceous material to drive 125 off phosphorus gas and carbon monoxid gas, feeding and conducting a stream of the phosphatic material and the flux toward the furnace, passing said phosphorus gas through said stream and admitting air to 130

said stream to effect a further oxidation of the phosphorus and the carbon monoxid while passing in said stream, and thereby pre-heating the material in said stream.

5. 4. The process of manufacturing phosphoric acid which consists in heating together in a furnace phosphatic material, a silicious flux and a carbonaceous material to produce phosphorus gas and carbon monoxid, leading said phosphorus gas and said monoxid in a current from the furnace, feeding and conducting a stream of the phosphatic material and the flux in a divided condition toward the furnace, revolving the said stream to effect its gradual progress toward the furnace, and introducing oxygen into said stream to oxidize the phosphorus to phosphorus pentoxid, and to oxidize the carbon monoxid to carbon dioxid within the stream, and thereby pre-heating the material in the stream before it passes into the furnace.

5. The process of manufacturing phosphoric acid which consists in heating together in a furnace phosphatic material, a silicious flux and a carbonaceous material to produce phosphorus gas and carbon monoxid, leading said phosphorus gas and said monoxid in a current from the furnace, feeding and conducting a stream of the phosphatic material and the flux through said current toward the furnace, revolving the said stream to effect its gradual progress toward the furnace, and introducing oxygen into said stream to oxidize the phosphorus to phosphorus pentoxid, and to oxidize the carbon monoxid to carbon dioxid within the stream, and thereby pre-heating the column before it passes into the furnace, and feeding a carbonaceous material into the furnace.

6. In an apparatus for producing phosphoric acid, in combination, a furnace for heating together a phosphatic material, a flux and a carbonaceous material, a duct through which gases from the furnace pass, means for feeding the phosphatic material and the flux to the furnace through said duct, said furnace having an inlet opening for admitting said carbonaceous material to the furnace hearth without passing the same through said duct.

7. In an apparatus for producing phosphoric acid, in combination, a furnace for heating together phosphatic material, a flux and a carbonaceous material to form phosphorus gas and carbon monoxid gas, a duct for conducting the phosphatic material and the flux into the furnace and through which the said gases pass, said duct constituting means for effecting the oxidation of said phosphorus and said carbon monoxid within said duct and thereby pre-heat the material in said duct as it passes to said furnace.

8. In an apparatus for producing phos-

phoric acid, in combination, a furnace for heating together phosphatic material, a flux and a carbonaceous material to form phosphorus gas and carbon monoxid gas, a duct for conducting the phosphatic material and the flux into the furnace and through which the said gases pass, said duct constituting means for effecting the oxidation of said phosphorus and said carbon monoxid within said duct and thereby pre-heat the material in said duct as it passes to said furnace, and means for rotating said duct to produce a thorough heating and mixture of the contents of said duct.

9. In an apparatus for producing phosphoric acid, in combination, a furnace for heating together phosphatic material, a flux and a carbonaceous material to form phosphorus gas and carbon monoxid gas, a duct for conducting the phosphatic material and the flux into the furnace and through which the said gases pass, said duct constituting means for effecting the oxidation of said phosphorus and said carbon monoxid within said duct and thereby pre-heat the material in said duct as it passes to said furnace, and means for admitting oxygen to said duct to effect the oxidation of said phosphorus gas and said carbon monoxid within said duct to pre-heat the material in said duct, and means for rotating said duct to produce a thorough heating and mixture of the contents thereof.

10. In an apparatus for producing phosphoric acid, a furnace for heating together phosphatic material, a flux, and a carbonaceous material, and thereby driving off oxidizable gases including phosphorus, means for holding a mass of the flux and the phosphatic material in a finely divided state and arranged so that the said oxidizable gases pass from the furnace through said mass, means for admitting air to effect the oxidation of the oxidizable gases while passing through said mass, and a filter arranged to receive the oxidized gases to remove the particles of dust carried thereby.

11. The process of manufacturing phosphoric acid which consists in heating together in a furnace phosphatic material, a flux, and a carbonaceous material to drive off oxidizable gases including phosphorus, preparing a charge for the furnace exclusive of the carbonaceous material, passing the gases from said furnace through said charge and thereby effecting the oxidation of the phosphorus in the gases as they pass through said charge to pre-heat the charge before it enters the furnace, and feeding carbonaceous material into the furnace.

12. The process of manufacturing phosphoric acid which consists in heating together in a furnace phosphatic material, a flux, and a carbonaceous material to drive off oxidizable gases including phosphorus, pre-

- paring a charge for the furnace exclusive of the carbonaceous material, passing the gases from said furnace through said charge and effecting the oxidation of the phosphorus 5 in the gases as they pass through said charge to pre-heat the charge before it enters the furnace, agitating the charge while the gases are passing through the same, and feeding carbonaceous material into the furnace.
- 10 13. The process of manufacturing phosphoric acid which consists in heating together in a furnace phosphatic material, a flux, and a carbonaceous material to drive off oxidizable gases including phosphorus, 15 preparing a charge for the furnace exclusive of the carbonaceous material, passing the gases from said furnace through said charge admitting air to effect the oxidation of the phosphorus in the gases as they pass through 20 said charge to pre-heat the charge before it enters the furnace, and feeding carbonaceous material into the furnace.
14. The process of manufacturing phosphoric acid which consists in heating together in a furnace phosphatic material, a flux and a carbonaceous material to drive off oxidizable gases including phosphorus, preparing a charge for the furnace including 25 the flux and the phosphatic material, passing the gases from said furnace through
- 30

said charge, admitting oxygen to effect the oxidation of the phosphorus gases as they pass through said charge to pre-heat the charge before it enters the furnace, collecting the dust from the gases after they pass 35 from the charge, and feeding carbonaceous material into the furnace.

15. The process of manufacturing phosphoric acid which consists in heating together in a furnace phosphatic material, a 40 flux and a carbonaceous material to drive off oxidizable gases including phosphorus, preparing a charge for the furnace including the flux and the phosphatic material in a finely divided state, passing the gases from said furnace through said charge, admitting oxygen to effect the oxidation of the phosphorus gases as they pass through said charge to pre-heat the charge before it enters the furnace, filtering the dust from the 45 gases after they pass from the charge, and feeding carbonaceous material into the furnace.

In testimony whereof I have hereunto set my hand in presence of two subscribing witnesses.

INGENUIN HECHENBLEIKNER.

Witnesses:

W. H. MARTIN, Jr.,  
E. C. MARSHALL.